

## 1

3,044,872

## STEEL ALLOY COMPOSITION

Walter C. Hayes, Northridge, and Robert W. Dickinson, Van Nuys, Calif., assignors to North American Aviation, Inc.

No Drawing. Filed Nov. 2, 1959, Ser. No. 850,117

3 Claims. (Cl. 75—126)

This invention relates to an improved high temperature alloy. More particularly, this invention relates to an improved high temperature steel alloy with low thermal coefficient of expansion, high thermal conductivity, and good high temperature mechanical properties.

Austenitic stainless steels are well known in the art. An example of a stainless steel is AISI type No. 304 which contains from 18% to 20% chromium and 8% to 11% nickel with 2% max. of manganese. It has a low carbon content and has many uses. However, it has some drawbacks, one of which is its relatively high cost because of the high chromium and nickel content. Also, its thermal coefficient of expansion is a little high for certain applications while its thermal conductivity is too low. On the other hand, ferritic steels have low coefficient of expansion and a high thermal conductivity as well as low cost but they are weak at elevated temperatures. Consequently, it would be advantageous to obtain a ferritic alloy which would combine the conductivity and expansion properties of ferritic steels with the excellent strength properties of austenitic steels for use at high temperatures. For such applications, high thermal conductivity, low thermal coefficient of expansion and, therefore, low thermal stresses are important.

It is, therefore, an object of this invention to provide a new steel alloy having high creep and stress rupture properties at elevated temperatures. It is also an object of this invention to provide a steel alloy having a high corrosion resistance in molten metal service. Another object of this invention is to provide a steel alloy having adequate strength and ductility in the heat-affected zone of weldments without costly post weld heat treatments. Another object of this invention is to provide a ferritic steel alloy having high temperature properties equal to or surpassing those of the austenitic steels. Still another object is to provide a steel alloy which is obtainable at a much lower cost than stainless steel. It is also an object to provide a steel alloy which has a low coefficient of expansion, a high thermal conductivity, and a high resistance to thermal stresses at elevated temperatures. Still other objects of this invention will become apparent from the discussion which follows.

The above and other objects of this invention are obtained by providing a steel alloy having improved high temperature properties containing from about 0.4% to about 10% chromium, from about 0.4% to about 4% molybdenum, from about 0.05% to about 0.4% carbon, from about 0.1% to about 1.5% manganese, from about 0.1% to about 1% niobium, from about 0% to about 1.4% titanium, from about 0% to about 4% nickel, and the remainder substantially iron. In addition, the alloy can contain about 0.1% (max.) boron, about 0.02% (max.) nitrogen, and about 0.2% (max.) aluminum, about 1.5% (max.) silicon, about 0.03% (max.) phosphorus, and about 0.03% (max.) sulfur.

Steel alloys having compositions falling within the range of components specified above are found useful in the fabrication of steam power plant components, such as piping systems for conveying high pressure and high temperature water and steam. They are also useful in the manufacture of high temperature steam heat exchangers as well as in the manufacture of pressure vessels to be used at high temperatures. Still other uses include piping systems, heat exchangers, and pressure vessels manufactured of these alloys for use in refineries where

## 2

the added strength over known stainless steels is beneficial.

The steel composition or alloys of this invention contain from about 0.4 to about 10 weight percent chromium in order to give the steel adequate corrosion and oxidation resistance. The steel alloys of this invention are particularly useful for service above about 1050° F. In order to assure oxidation resistance at temperatures of this magnitude it is preferred to include at least about 1.5 weight percent chromium. This constitutes a preferred minimum chromium concentration. One of the properties of the steel alloy of this invention is good notched impact properties at high temperatures. It is found that these are not enhanced to any appreciable degree by chromium concentrations above about 7.5 weight percent and, therefore, the latter amount constitutes a preferred upper limit to the chromium concentration. Hence, the preferred range of chromium is from about 1.5 weight percent to about 7 weight percent.

20 The molybdenum concentration in the steel alloys of this invention varies from about 0.4 to about 4 weight percent. An amount of molybdenum equivalent to about 0.4 weight percent together with the amount of chromium indicated above is sufficient to impart a perceptible degree of resistance to oxidation and a fair degree of strengthening at elevated temperatures. The 0.4 weight percent, therefore, constitutes a preferred lower limit for the molybdenum content. No additional benefit is obtained from amounts of molybdenum above about 4 weight percent and the latter, therefore, constitutes an upper limit of the molybdenum concentration.

The carbon is present in the novel steel alloys in amounts ranging from about 0.05 to about 0.4 weight percent in order to impart strengthening characteristics to the steel. At least about 0.05 weight percent carbon is required in order to impart a discernible increase in the strength of the steel. Above about 0.4 weight percent carbon there is a danger of making the steel too brittle. The broad range of carbon concentrations, therefore, varies in the range of from about 0.05 to about 0.4 weight percent. However, in order to obtain an increase in the strength of the steel of practical magnitudes, it is preferred to have at least about 0.08 weight percent carbon. Also, in order to minimize the degree of embrittlement imparted to the steel, it is preferred to limit the total carbon to about 0.3 weight percent. Thus, the preferred carbon concentration is about 0.08 weight percent to about 0.3 weight percent.

It has been found that the addition of from about 0.1 to about 1 weight percent niobium to the above described steels containing chromium, molybdenum, and carbon in the amounts indicated, imparts a high degree of strength increase at elevated temperatures. With the added niobium, the resulting steel has a low notch sensitivity in stress rupture tests at elevated temperatures. It also exhibits good notched impact properties at ambient (room) temperature. The degree of strengthening due to the columbium becomes effectively significant at a concentration of about 0.1 weight percent niobium. The beneficial strengthening effect decreases rapidly per increment of niobium added above about 1 weight percent. Therefore, the preferred range of niobium concentration in the steel alloy of this invention varies from about 0.1 to about 1 weight percent.

65 Many steels contain titanium which functions as a grain refining element and a strengthening agent. It is found that the addition of niobium to titanium-containing steels in which the amounts of chromium, molybdenum, and carbon are as stated hereinabove, greatly increases the high strength property of the steel. Usually about 0.1 weight percent titanium is added to the steel in order to achieve a significant effect in the elevated temperature

mechanical properties. Above about 1.4 weight percent titanium it is found that the quality of the steel is not improved to any significant degree and, therefore, the titanium content varies from about 0.1 to about 1.4 weight percent in one embodiment of the steel alloy of this invention. To the titanium-containing steel alloy can be added from about 0.1 to about 1 weight percent niobium to increase the elevated temperature strength of the alloy as stated hereinabove. It is, however, found that optimum strengthening properties are obtained when the total amount of the added niobium and titanium varies from about 0.2 to about 1.5 weight percent and wherein the amount of niobium is from about 0.1 weight percent to about 1 weight percent, and this constitutes a preferred embodiment of this invention.

Nickel is added to steel in order to lower the minimum temperature required for solution heat treating, and to improve low temperature ductility and impact strength. Amounts of nickel ranging from about 0.1 to about 4 weight percent give satisfactory results in the solution heat treating of the steel alloy compositions of this invention. At least about 0.1 weight percent of nickel is required in order to give a significantly perceptible effect, while amounts above about 4 weight percent of nickel decrease the response to heat treatment. The addition of niobium to a nickel-containing steel alloy having chromium, molybdenum, and carbon in the amounts outlined hereinabove, substantially increases the elevated temperature strength of the steel. The amount of niobium added in this instance is the same as that added to the other niobium-containing steel embodiments of this invention. In other words, the chromium, molybdenum, carbon, and nickel-containing steel as hereinabove specified can contain from about 0.1 to about 1 weight percent niobium. This, then, constitutes another embodiment of the instant invention.

Still another embodiment of this invention is a steel alloy composition containing the chromium, molybdenum, carbon, and nickel in the amounts specified hereinabove together with titanium and niobium in an amount varying from about 0.2 to about 1.5 weight percent wherein the amount of niobium varies from about 0.1 to about 1 weight percent. This composition then has the properties of a similar composition minus nickel described hereinabove as well as the added advantage of having a lowered solution heat treating temperature. The nickel-, titanium-, and niobium-containing alloy, therefore, constitutes still another embodiment of this invention.

By elevated temperature strength in the above discussion is meant the strength at temperatures above about 1050° F. In addition to the high temperature strength, the alloys of this composition also have the added advantage of low cost, good general corrosion resistance, resistance to chloride stress corrosion, good weldability, and good resistance to thermal stresses.

In general, a heat of steel of this invention is melted and cast by conventional methods. The cast metal can be hot worked by conventional practices to a wrought product. Heat treatment is accomplished by heating to from about 1800° F. to about 2200° F. for a period of from about 0.5 to about 10 hours. Following this, the metal alloy is air cooled or quenched to a temperature of from about 1300° F. to about 0° F. This is followed by aging or tempering at a temperature of from about 1100° F. to about 1400° F. for a period of from about 0.5 to about 24 hours. This treatment results in a steel alloy which is more ductile and less notch sensitive than ordinary high chromium-containing steels.

The following non-limiting examples further illustrate the various steel alloy compositions of this invention.

#### EXAMPLE

25 An induction heat was air melted and cast into a hot topped 4 1/4" square tapered ingot. A chemical analysis of the ingot showed substantially the following composition in percentage by weight: 2.32% chromium, 1.09% molybdenum, 0.47% titanium, 0.13% carbon, 0.49% manganese, 0.37% niobium, 0.009% phosphorus, 0.022% sulfur, 0.21% silicon, 0.006% nitrogen, 0.002% aluminum, and the balance substantially iron. The ingot was hot-rolled to form a 3/4" plate with a reduction ratio of approximately 5-to-1. The steel was heated to 2100° F. for a period of 1 hour followed by air cooling to a temperature of substantially 70° F. It was then heated to a temperature of substantially 1300° F. for a period of 8 hours, and then cooled to 70° F.

#### EXAMPLE II

Following the procedure of Example I, a heat having the following composition was processed: 2.42% chromium, 1.04% molybdenum, 0.14% carbon, 0.5% manganese, 0.12% niobium, 0.35% titanium, 0.008% phosphorus, 0.024% sulfur, 0.20% silicon, 0.006% nitrogen, 0.004% aluminum, and the balance substantially iron.

Still other steel alloys of this invention and their composition are given in the following Table I. The balance

Table I

| Heat No. | Cr   | Mo   | C    | Mn   | Nb   | Ti   | Ni   | B, Max. | N, Max. | Al, Max. | Si, Max. | P, Max. | S, Max. |
|----------|------|------|------|------|------|------|------|---------|---------|----------|----------|---------|---------|
| 1        | 0.4  | 0.4  | 0.05 | 0.1  | 0.1  | 0    | 0    | 0.02    | 0.2     | 1.5      | 0.03     | 0.03    |         |
| 2        | 0.4  | 0.4  | 0.05 | 0.1  | 0.1  | 0.1  | 0    | 0.02    | 0.2     | 1.5      | 0.03     | 0.03    |         |
| 3        | 0.4  | 0.4  | 0.05 | 0.1  | 0.1  | 0.1  | 0.1  | 0.02    | 0.2     | 1.5      | 0.03     | 0.03    |         |
| 4        | 10   | 4    | 0.4  | 1.5  | 1    | 1.4  | 4    | 0.1     | 0.02    | 0.2      | 1.5      | 0.03    | 0.03    |
| 5        | 10   | 4    | 0.4  | 1.5  | 1    | 0    | 0    | 0.1     | 0.02    | 0.2      | 1.5      | 0.03    | 0.03    |
| 6        | 10   | 4    | 0.4  | 1.5  | 1    | 0.4  | 0    | 0.1     | 0.02    | 0.2      | 1.5      | 0.03    | 0.03    |
| 7        | 10   | 4    | 0.4  | 1.5  | 1    | 0.4  | 4    | 0.1     | 0.02    | 0.2      | 1.5      | 0.03    | 0.03    |
| 8        | 1.5  | 0.4  | 0.08 | 0.1  | 0.1  | 0    | 0    | 0.02    | 0.2     | 1.5      | 0.03     | 0.03    |         |
| 9        | 1.5  | 0.4  | 0.08 | 0.1  | 0.1  | 0.1  | 0    | 0.1     | 0.02    | 0.2      | 1.5      | 0.03    | 0.03    |
| 10       | 1.5  | 0.4  | 0.08 | 0.1  | 0.1  | 0.1  | 0.1  | 0.1     | 0.02    | 0.2      | 1.5      | 0.03    | 0.03    |
| 11       | 7.5  | 4    | 0.3  | 1.5  | 1    | 1.4  | 4    | 0.1     | 0.02    | 0.2      | 1.5      | 0.03    | 0.03    |
| 12       | 7.5  | 4    | 0.3  | 1.5  | 1    | 0    | 0    | 0.1     | 0.02    | 0.2      | 1.5      | 0.03    | 0.03    |
| 13       | 7.5  | 4    | 0.3  | 1.5  | 1    | 0.4  | 0    | 0.1     | 0.02    | 0.2      | 1.5      | 0.03    | 0.03    |
| 14       | 7.5  | 4    | 0.3  | 1.5  | 1    | 0.4  | 4    | 0.1     | 0.02    | 0.2      | 1.5      | 0.03    | 0.03    |
| 15       | 0.4  | 0.4  | 0.05 | 0.1  | 0.1  | 1.4  | 0    | 0.1     | 0.02    | 0.2      | 1.5      | 0.03    | 0.03    |
| 16       | 10   | 4    | 0.4  | 1.5  | 1    | 0.5  | 0    | 0.1     | 0.02    | 0.2      | 1.5      | 0.03    | 0.03    |
| 17       | 1.5  | 0.4  | 0.08 | 0.1  | 0.1  | 1.4  | 0    | 0.1     | 0.02    | 0.2      | 1.5      | 0.03    | 0.03    |
| 18       | 1.5  | 0.4  | 0.08 | 0.1  | 1    | 0.5  | 0    | 0.1     | 0.02    | 0.2      | 1.5      | 0.03    | 0.03    |
| 19       | 7.5  | 4    | 0.3  | 1.5  | 1    | 0.5  | 0    | 0.1     | 0.02    | 0.2      | 1.5      | 0.03    | 0.03    |
| 20       | 10   | 4    | 0.4  | 1.5  | 1    | 0.5  | 4    | 0.1     | 0.02    | 0.2      | 1.5      | 0.03    | 0.03    |
| 21       | 7.5  | 4    | 0.3  | 1.5  | 1    | 0.5  | 4    | 0.1     | 0.02    | 0.2      | 1.5      | 0.03    | 0.03    |
| 22       | 0.4  | 0.4  | 0.05 | 0.1  | 0.1  | 0    | 0.1  | 0.02    | 0.2     | 1.5      | 0.03     | 0.03    |         |
| 23       | 10   | 4    | 0.4  | 1.5  | 1    | 0    | 4    | 0.1     | 0.02    | 0.2      | 1.5      | 0.03    | 0.03    |
| 24       | 1.5  | 0.4  | 0.08 | 0.1  | 0.1  | 0    | 0.1  | 0.02    | 0.2     | 1.5      | 0.03     | 0.03    |         |
| 25       | 7.5  | 4    | 0.3  | 1.5  | 1    | 0    | 4    | 0.1     | 0.02    | 0.2      | 1.5      | 0.03    | 0.03    |
| 26       | 2.25 | 1    | 0.15 | 0.5  | 0.4  | 0.4  | 0    | 0.1     | 0.02    | 0.2      | 1.5      | 0.03    | 0.03    |
| 27       | 2.3  | 1.07 | 0.15 | 0.49 | 0.40 | 0.47 | 0    | 0.0007  | 0.006   | 0.06     | 0.46     | 0.018   | 0.023   |
| 28       | 2.3  | 1    | 0.16 | 0.6  | 0.8  | 0    | 0    | 0.0006  | .008    | .07      | 0.4      | 0.02    | 0.025   |
| 29       | 2.2  | 2    | 0.14 | 0.3  | 0.45 | 0.35 | 0    | 0.0009  | .005    | .05      | 0.35     | 0.015   | 0.02    |
| 30       | 5    | 1    | 0.2  | 0.6  | 0.49 | 0.37 | 0    | 0.0008  | .013    | .09      | 0.6      | 0.01    | 0.016   |
| 31       | 2.28 | 1.1  | 0.14 | 0.48 | 0.46 | 0.34 | 1.28 | 0.0006  | 0.009   | .08      | 0.38     | 0.021   | 0.019   |
| 32       | 2.15 | 1.23 | 0.15 | 0.4  | 0.32 | 0.47 | 0    | 0.0008  | .004    | .06      | 0.41     | 0.02    | 0.02    |

of the composition in each heat is substantially iron. Tables II and III show the various properties of a steel alloy of this invention together with the properties of ferritic steel and 304 stainless steel for comparison purposes.

Table II

| Alloy (Wt. Percent)                                  | Tensile Properties (at Room Temperature)            |                                                    |
|------------------------------------------------------|-----------------------------------------------------|----------------------------------------------------|
|                                                      | 0.2% Offset Yield Strength (10 <sup>3</sup> p.s.i.) | Ultimate Tensile Strength (10 <sup>3</sup> p.s.i.) |
| Fe+2.25 Cr+1 Mo+0.4 Ti+0.4 Nb                        | 93.0                                                | 108.0                                              |
| Fe+2.25 Cr+1 Mo                                      | 41.5                                                | 79.9                                               |
| Type 304 Stainless Steel                             | 37.2                                                | 85.2                                               |
| Short Time Tensile Properties (at 1,050° F.-565° C.) |                                                     |                                                    |
| Fe+2.25 Cr+1 Mo+0.4 Ti+0.4 Nb                        | 67.0                                                | 71.0                                               |
| Fe+2.25 Cr+1 Mo                                      | 27.1                                                | 50.2                                               |
| Type 304 Stainless Steel                             | 14.0                                                | 55.0                                               |
| Short Time Tensile Properties (at 1,200° F.-650° C.) |                                                     |                                                    |
| Fe+2.25 Cr+1 Mo+0.4 Ti+0.4 Nb                        | 56.0                                                | 60.0                                               |
| Fe+2.25 Cr+1 Mo                                      | 18.3                                                | 32.9                                               |
| Type 304 Stainless Steel                             | 12.0                                                | 48.0                                               |

Table III

| Alloy (Wt. Percent)           | Min. Creep Rates (at 1,050° F.-565° C.) |                                  | Stress to Rupture (at 1,100° F.-593° C.) |                        |
|-------------------------------|-----------------------------------------|----------------------------------|------------------------------------------|------------------------|
|                               | Stress 10 <sup>3</sup> p.s.i.           | Min. Creep, Rate Percent Per Hr. | Time in hours                            | 10 <sup>3</sup> p.s.i. |
| Fe+2.25 Cr+1 Mo+0.4 Ti+0.4 Nb | 7.5                                     | 5×10 <sup>-6</sup>               | 10                                       | 48                     |
|                               | 12.5                                    | 2.5×10 <sup>-5</sup>             | 100                                      | 40                     |
|                               | 17.5                                    | 1.0×10 <sup>-4</sup>             | 1,000                                    | 33                     |
|                               | 25.0                                    | 1.0×10 <sup>-3</sup>             | 10,000                                   | 26                     |
|                               | 7.5                                     | Less than 10 <sup>-6</sup>       | 10                                       | 45                     |
|                               | 12.5                                    | 3.5×10 <sup>-5</sup>             | 100                                      | 32                     |
| Type 304 Stainless Steel      | 17.5                                    | 3.5×10 <sup>-4</sup>             | 1,000                                    | 23                     |
|                               | 25.0                                    | 5.5×10 <sup>-3</sup>             | 10,000                                   | 17                     |
|                               | 7.5                                     | 5×10 <sup>-5</sup>               | 10                                       | 27                     |
|                               | 12.5                                    | 4×10 <sup>-4</sup>               | 100                                      | 20                     |
| Fe+2.25 Cr+1 Mo               | 17.5                                    | 2×10 <sup>-3</sup>               | 1,000                                    | 45                     |
|                               |                                         |                                  | 10,000                                   | 10.3                   |

The chemical analysis of the steel alloy of this invention given in Table II and III as Fe+2.25 Cr+1 Mo+0.4 Ti+0.4 Nb is that given for heat No. 27 in Table I, supra. It will be noticed from Table III that the alloy of this invention requires from about 6.7% to about 53% higher stress to rupture in the same time as that required for the rupture of 304 stainless steel, and from about 78% to about 152% higher stress than required for the rupture of ferritic steel containing 2.25 weight percent chromium and 1 weight percent molybdenum. That is, by merely adding a small amount of niobium and titanium, the composition of the steel is improved with respect to stress to rupture by 152%. From Table II it is seen that the offset yield strength of the niobium-containing alloy of this invention is 124% higher than that of 2.25% chromium and 1% molybdenum ferritic steel and 150% higher than that of 304 stainless steel at room temperature; 147% higher than that of ferritic steel and 378% higher than that of stainless steel at 1050° F. (565° C.); and 206% higher than ferritic steel and 366% higher than stainless steel at 1200° F. (650° C.). It is also seen that the ultimate tensile strength of the niobium-containing steel is 35% higher than that of ferritic steel and 26% higher than that of stainless steel at room temperature; 41% higher than

that of ferritic steel and 29% higher than that of stainless steel at 1050° F.; and 82% higher than that of ferritic steel and 25% higher than that of stainless steel at 1200° F. From Table III it is also noted that the minimum 5 creep rate of the niobium-containing steel of this invention is from about a factor of 2 to about a factor of 10 lower than for ferritic steel and from about a factor of 5 to about a factor of 10 lower than that of the 304 stainless steel. Thus components manufactured from the 10 steel alloys of this invention will deform only at very slow rates when in highly stressed service at temperatures up to at least about 1100° F.

The steel alloy specimens of this invention used for the tests given in Tables II and III were 4 inches long with a 1.5 inch gauge length and a gauge diameter of 0.375 inch. The specimen steel alloys of this invention described in the Examples and in Table I, like the specimen used to illustrate the improvement in the properties listed in Tables II and III, all have properties which are 15 an improvement over the ferritic and stainless steel compositions.

While the invention has been described with reference to specific steel alloy compositions, it is to be understood that this is by way of example only and not by way of limitation. The spirit and scope of the invention is to be 20 limited only by the appended claims.

We claim:

1. An alloy having improved high temperature properties consisting essentially of—

30 from about 0.4% to about 7.5% chromium  
from about 0.4% to about 4.0% molybdenum  
from about 0.05% to about 0.4% carbon  
from about 0.1% to about 1.5% manganese  
from about 0.1% to about 1.0% niobium  
from about 0.1% to about 1.4% titanium  
and the remainder essentially iron.

2. An alloy having improved high temperature properties consisting essentially of—

35 from about 2.0% to less than 4.0% chromium  
from about 1.0% to about 2.0% molybdenum  
from about 0.05% to about 0.4% carbon  
from about 0.1% to about 1.5% manganese  
from about 0.1% to about 1.0% niobium  
from about 0.1% to about 1.4% titanium  
and the remainder essentially iron.

3. An alloy having improved high temperature properties consisting essentially of—

40 about 2.25% chromium  
about 1.0% molybdenum  
about 0.15% carbon  
about 0.5% manganese  
about 0.4% niobium  
about 0.4% titanium  
about 0.1% (max.) boron  
about 0.02% (max.) nitrogen  
about 0.2% (max.) aluminum  
about 1.5% (max.) silicon  
about 0.03% (max.) phosphorus  
about 0.03% (max.) sulfur  
and the remainder essentially iron.

#### References Cited in the file of this patent

#### UNITED STATES PATENTS

- 2,159,723 Franks May 23, 1939  
2,194,178 Becket et al. Mar. 19, 1940  
2,513,935 Harris July 4, 1950  
2,590,835 Kirkby et al. Apr. 1, 1952  
2,905,577 Harris et al. Sept. 22, 1959